

Feb. 17, 1931.

A. THOMA

1,793,340

SHOE BOTTOM FILLER PIECE

Filed Aug. 6. 1928



Patented Feb. 17, 1931

1,793,340

# UNITED STATES PATENT OFFICE

ANDREW THOMA, OF CAMBRIDGE, MASSACHUSETTS, ASSIGNOR TO NORTH AMERICAN CHEMICAL COMPANY, OF BOSTON, MASSACHUSETTS, A CORPORATION OF MASSACHUSETTS

## SHOE-BOTTOM FILLER PIECE

Application filed August 6, 1928. Serial No. 297,630.

This invention relates particularly to the provision of shoe-bottom filler in permanent sheet-like form and coherent, durable units or pieces of standardized shapes or areas and volumes as articles of manufacture, standardized in accordance with the sizes and shapes of the shoes or other preferences of the trade and of different shoe manufacturers, and capable of being shipped, stored and handled and yet ready for instant use (including treatment if necessary), whenever and however required for the shoe filling operation. The present application is the foundation application of a series, all relating to this invention considered broadly, and discloses and claims the invention generally, which consists, generically or broadly stated, of the predetermined or standardized pieces or units explained, each containing a predetermined quantity of filler material required to fill the shoe-bottom cavity, and a predetermined contour less in size and shape than the cavity, but greater in thickness than the depth of said cavity, said pieces being spreadable in use in whatever direction required to fill the cavity properly, but compacted, supported and retained sufficiently as a whole to be stable and shape-maintaining under commercial conditions of handling and shipping prior to use. To the latter end the pieces have durable, non-sticky, unified exteriors for self-preservation during transportation and storage, but both as to interior and exterior their structure and composition is subject to wide variation. In the present application I have not undertaken to set forth, except in a general way, the many species or variations of pieces within the broader concept and embodiment of the invention, as the same is further fully set forth in the various copending applications of the aforesaid series, and particularly in application Ser. No. 133,506 filed Sept. 3, 1926, of which the present application is a continuation in part, and where the invention, considered broadly is set forth at length, together with claims for the species which employs external means constituting a cover, stiffener, shape retainer, carrier-support or the like

on one or both sides, besides certain other less prominent features.

The primary object is to simplify and cheapen the filling process by doing away with the expensive machines now required for preparing and applying the common, plastic, bulk filler in welt shoe manufacture, by providing, as articles of manufacture, the filler units ready-made or self-contained and durable in quantity, shape, character and condition, so that the former skill, time, and expense are largely eliminated, as all the operator has to do is to place the piece in the shoe cavity, first heating or conditioning it if required. For McKay shoe manufacture my invention opens the way to the practicable use of the same spreadable filler which has always heretofore been restricted to welt shoe manufacture.

The broad invention consists of the standardized units or pieces explained, each made as a layer which is sufficiently dense, unified and compacted as a whole to be shape-sustaining and self-maintaining, but yet spreadable, self-shaping and adhesive when laid in the shoe-bottom and subjected to levelling pressure or to the usual pressure of the spatula in the hands of the operator, and externally durable, non-adhesive and handleable for shipping, storage and usual commercial handling. In use also it is non-stretchable and non-shrinkable, or in other words is stable and tough while yet sufficiently pliable and yielding to be comfortable to the foot of the wearer. While I disclose and claim hereinafter a particular species, the main body of the piece, for general purposes, and as covered by the broader claims herein, may consist of or contain filler material, preferably of the plastic kinds or compositions set forth in my various plastic filler Patent No. 832,002, dated September 25, 1906; 855,868, dated June 4, 1907 and subsequent patents, and the copending filler applications already referred to. The numerous patents and concurrent applications above mentioned disclose a wide variety of shoe filler materials, mostly plastic and moldable, some normally sticky, some requiring heat or other treatment to become sticky or adhesive, some being

inherently stable, coherent, and cohesive, others not so, some being granular, others not granular, and so on to meet all situations of the shoe filling art. The chief of said fillers is 5 the spreadable one composed mainly of residuum of petroleum or other meltable or plastic binder, intermixed with ground cork or other comminuted material. All these fillers were previously made and shipped in bulk 10 to the shoe factory and there reduced by melting or otherwise to a shapeless but spreadable mass to be laid in the shoe-bottom with a spatula as a mason lays mortar with a trowel. My present invention contemplates 15 the use of any of the foregoing fillers, but in a radically different manner and embodiment. Instead of a shapeless mass and indefinite volume, the filler is sheeted or molded and compressed into coherent, granular units of 20 standardized shape and volume adapted, as articles of manufacture, to fill the general run of shoes, so as not to need cutting and trimming for each individual shoe, each unit having the predetermined volume suitable for 25 filling a single shoe-bottom cavity. The shiftability or spreadability of this unit is held in check or inoperative in the standardized pieces so that they do not stick to each other or change shape or character, but are readily 30 transported and remain neutral to each other and to surroundings until used, whereupon the inherent spreadability becomes or is made active and is then relied upon mainly for the final automatic fitting of the piece or unit 35 to the cavity, preferably accomplished by pressure, preferably the levelling pressure. My invention is intended for welt shoes and McKay shoes, but particularly the latter. It has heretofore been considered impracticable 40 to make McKay shoes with a spread or plastic-laid filler, but my present invention makes this practicable. The unit or piece is made of predetermined dimensions different from those of the cavity being thicker than the 45 cavity depth and less in area than the cavity area, and therefore capable of being spread after being placed in the shoe-bottom to the shape and to the reduced thickness and increased area required for substantially filling 50 said cavity to the extent commonly required by McKay shoe manufacturers, and to at least the extent as practiced and understood by said shoe makers as filling the bottoms of McKay shoes. These units are first 55 made in a large sheet fabric or layer which is flexible, waterproof, moldable, dense, durable, coherent and self-sustaining for shipping and handling. In other words it contains such shoe filler characteristics as are 60 possessed by the particular variety of shoe filler used, and in addition thereto it is in a sheet or fabricated layer having the durable, handleable qualities necessary for commercial requirements while preserving said filler 65 characteristics dormant but ready for instant use when required for the shoe filling operation. Then at the filler manufactory it is subdivided into the aforesaid units or distinct, individual, standard pieces, entirely ready for subsequent use individually and in quantity at the shoe factory. Preferably one side, or it may be both sides of the plastic unit or above fabricated layer piece has a supporting, protecting, or shape-retaining layer, as set forth in further detail and duly claimed in 70 my application 133,506 filed September 3, 1926. If such a cover layer is on one side only, the other side is preferably dusted, impregnated, or dulled with various powders, dry fibrous materials, ground cork or the like, 75 pressed into or incorporated on and embedded into the surface of the plastic layer sufficiently to protect it in being handled, transported and until its time of use for filling the shoes, and constituting a resurfacing of the unit or 80 piece as more fully set forth and claimed specifically in my application Ser. No. 183,302, filed April 13, 1927. In any case, the sticky layer, or the spreadable layer of filler material, is so protected, constructed, or related 85 that it, or the piece or filler article of which it is a part, is capable of being handled integral 90 and placed as an integral, self-maintaining piece in the shoe cavity. It is then spread as stated. It is capable of sticking in 95 place as a piece with its own inherent stickiness or may contain special external adhesive, and in either case the stickiness may be temporarily held inactive. The method of use in 100 certain respects noted above is contained in my copending applications Ser. No. 210,558, filed August 4, 1927 and Ser. No. 242,085, filed December 23, 1927.

When the main body of filler material is enclosed by outside protectors or covers, I 105 preferably provide a considerable looseness or slight instability of the inner granular layer of cork or other comminuted body material. The mixture of comminuted body material and binder constituting the plastic 110 filler mixture is sheeted between hot rolls or otherwise reduced to the desired thin layered condition just as it is laid or delivered between the webs of paper, paper-like material, or other fabric, and then when cooled the 115 composite layer or more or less soft and pliable sheet may be compressed to a firmer, stronger consistency. The binder and cementing agent of the granular mass binds said mass together and also binds the mass 120 and the paper together as one whole laminated structure. This pad-like sheet is then 125 died into the small pieces required, which may be of almost any shape desired. As the spreadability of the piece is relied upon for the complete, perfect filling of the shoe-bottom cavity, it is not necessary that the shape of the piece should conform to the shape of the cavity.

Instead of a laminated piece in the sense 130

of having one or more separate layers of paper or other sheeted protector, the stand-ardized piece may be, and preferably is, made as a single, substantially homogeneous layer. 5 I have found asphalts especially advanta-geous for this purpose. I have found that such a homogeneous piece consisting solely of blown asphalt i. e. consisting of residuum of petroleum of the asphaltic base treated 10 until it is substantially saturated with oxygen or at least until its character is changed into permanent flexibility or pliability so as to eliminate its natural brittleness by being toughened by oxygenating treatment to the 15 extent known by the name of blown asphalt; has remarkable and unexpected advantages in carrying out my invention. Such a piece is non-sticky externally as an article of manu-facture, softens and readily becomes spread-able and under the sudden high heat treat-ment hereinafter explained, becomes perma-nently pliable when thus laid in the shoe bottom, never becomes liable to bunch, is very 20 strongly adherent to leather, so that the blown 25 asphalt layer can never shift in the shoe bottom, is not responsive so as to soften under any heat to which the shoe would be exposed in use, is tough and durable beyond the ordi-nary life of the shoe, needs no backer or 30 strengthening element as a filler component within or on the piece, is cheap, without waste in manufacture and use and is always clean. The wax tailings binder of my pre-vious patents is of a paraffin base, low melt-ing, sticky and unchangeable, and has as one 35 of its most valuable characteristics an oily nature which makes the material very tract-able by not sticking to the heated laying tool, and therefore is readily and easily applied 40 to the shoe-bottom. On account, however, of its low melting nature, it has always had a tendency to "bunch" and therefore a num-ber of my patents have to do with various restraining agents whose purpose has been 45 to make the low melting element firm or altered by the pasty restrainer after laying, so as not thereafter to be so liable to shift or be heat responsive. Asphalts, on the other hand, particularly those derived from pe-troleum residuum of a bituminous base, set 50 more permanently, but have a strong tend-ency to smouch or stain, and, lacking the oily paraffin-like nature, cling or stick to the filler knife, so that in the filler, as heretofore made 55 and used, it was impracticable and in fact impossible to use this clinging, smouching asphalt. But by having the filler delivered to the operator in a fully finished, predeter-mined piece, requiring simply to be placed 60 in the shoe-bottom hot and then simply pressed down and spread outwardly, as will be better understood from later disclosures, there is no longer any danger of smouching and staining, inasmuch as the operator does 65 not dip a flowing mass and hence cannot drop 70 particles therefrom, and the clinging ten-dency, under the method hereinafter set forth, becomes an advantage instead of a disad-vantage. Asphalt materials can be purchased of a far greater variety than wax tailings and 75 having a higher melting nature, greater tenacity, and flexibility, possessing a denser, more viscous body, or in other words, they give to the filler piece greater body and bind-ing capacity in conjunction with fibrous or 80 granulated body materials. Because of their high melting point, a filler mixture of body material and these dense-body asphalts of 180°-200° Fahrenheit melting point could not be used in mass in a kettle or usual filler appa-ratus as now done with present plastic fillers 85 because it would expose the operator to an unbearable heat and heat conditions absolutely impossible for him to endure day after day in his regular work in the shoe factory. The 90 objectionable heat and the greater muscular force which would be necessary in preparing, applying and manipulating the same in the usual hand operations, renders such use of this desirable material in the old mass-em-bodiment and old method impossible. 95

For best results I use an oxygenated as-phalt or "blown asphalt", as it is known in the market, (which is an asphalt derived from residuum of petroleum) of about 180°-200° 100 Fahrenheit melting point, and add thereto under proper fluxing or mixing heat (which, because of the mechanical force of the power mixed, need not be nearly as high as said melt-ing point) finely decimated woody matter such as cork, sawdust, charcoal or any vegeta-ble mass. This produces a rubber-like mass. For more leather-like material I use in con-junction with the aforesaid bulk-giving ma-terials, fibrous matter to impart to the mass 105 strength, toughness and tenacity. Also the blown asphalt is an especially rubber-like and leather-like pitchy material. By subjecting this to pressure and especially rolling pres-sure, I secure such degree of compactness as is 110 desired. Wood dust, powdered minerals, and powdered fibrous matter, one or all, added, give a still stiffer product when the whole 115 is sheeted into the finished article. The ingre-dients are mixed to the consistency of a flexible mass, consisting approxi-mately of binder one part in bulk, which is 120 principally blown asphalt of 180°-200° Fah-renheit melting point, or thereabouts, and two parts in bulk of the fine body material, and then sheeted between rolls and layers or webs of wet canvas to the desired thickness. This hot and otherwise semi-sticky mass is readily 125 sheeted, controlled and manipulated between the wet surfaces of the two canvas layers, which cause it quite readily to congeal as it is exposed to the cold moisture and the atmos-phere. When withdrawn from the wet can-130

vas, the sheeted layer is in a compact form which can then be subjected to further rolling pressure. The outside surfaces are now no longer sticky but can be handled with impunity. Furthermore the second treatment 5 has given the outside a thin but tough and relatively hard skin of almost clear binder. It is then cut or died into the particular shape chosen for the standard filler pieces in quantity.

10 At the shoe factory the operator has a small hot plate, gas or electric, which he keeps at a high heat. He takes two, three, or more spreading knives or spatulas, according to his 15 speed, places one filler piece on each knife, and lays the knives with their blades flat on the high-heat hot-plate. The filler piece is very quickly brought to a readily spreadable condition. The operator then takes a shoe 20 in his left hand, bottom up, lifts the first knife with his right hand, turns it over so as to bring the knife on top with the piece suspended therefrom over the bottom cavity of the shoe, and instantly places the piece and 25 spreads it in the shoe cavity. He then puts another piece on said knife and places it on the hot plate as before, takes up the second shoe, the second knife and its now melted piece, and repeats the reversal process and 30 spreading operation. He then places a fresh piece on this now empty second knife and puts it on the hot plate, takes the third knife and melted piece and fills the third shoe. And so on, rapidly and with extreme ease, 35 neatness and accuracy. If the operator is extremely rapid he may keep five knives, for instance, in use; if he is slow, two knives, for example. This all depends on the time required for melting a piece. By reason of my 40 process or method, the high heat is not destructive of the piece. The dry piece does not come in direct contact with the high heat as the cold or cooled knife is between the high heat plate and the piece, and although the 45 knife, being quite thin, very quickly attains substantially the same high heat as the plate, the short interval of less heat has permitted the dry piece to become moist or melted against the knife and hence self-protecting 50 against burning or charring. Also the outer skin, as stated, is practically clear binder and hence at once responsive to the high heat. But my method insures against charring even though some granules of the granulated cork 55 or other readily burned body material should happen to be in or on the surface of the piece. The asphalt, even if of the same low melting quality as the slippery, oily paraffin-base wax tailings previously mentioned, and particu- 60 larly if of the blown asphalt character, and still more particularly if of the high melting point grade of asphalt mentioned, has not only an absence of said slippery character when melted, but has enough tackiness or adhesiveness to cling to the knife sufficiently to

70 permit the reversal of the knife and piece to bottom-side-up position to permit the laying of the piece properly in the shoe-bottom cavity, as explained above. As a practical matter, this is an important element in the speed, accuracy and efficiency of this new method. The spatula or the spreading tool thus becomes a holding tool, heating tool, and a levelling tool.

75 A further refinement of this filler piece which I have last explained, resides in employing in the binder divergent elements which are reluctant to mix or coalesce with each other. For example, the residuums or suitable by-products of a paraffin base can be easily selected with a different degree of penetration from the residuums of an asphalt base. Although both are derived from petroleum, yet those varieties from the paraffin base are usually oily, as already stated, 80 and especially if such as petrolatum is used, whereas the available materials from the asphalt base lack this greasy quality and are not slippery but are dense, tough and tacky when melted, as already explained, and therefore only slightly penetrative and reluctant to coalesce with the paraffin base elements mentioned. Likewise I select body materials which are widely divergent in absorptive properties. For instance ground 85 cork, palm fibres and various other similar materials are not absorptive, or only slightly so, whereas sawdust, leather dust, wood pulp and various other filler materials are highly absorptive. Accordingly these filler materials of divergent absorptive properties are mixed in accordance with the selection and proportions of binder materials so as to co-operate with the selection made of penetrative and non-penetrative elements aforesaid. 90 The binder is compounded as aforesaid for spreading purposes and to make it easier for the operator. The petrolatum, using this as the best illustration so far mentioned, being finely distributed among the finely distributed sticky element, (asphalt), controls and lowers the melting point and likewise gives a smooth, easy, immediate spreading to the filler, and then at once the absorptive element in the body material withdraws from the binder the softer element, i. e. lower melted element, from the binder by absorption, leaving the higher melting or stiffer setting element substantially alone as the final binder to stiffen and render firm the set layer with all its natural or unmodified stiffness. Instead of petrolatum, various oils, greases or fats or combinations thereof may be used. The object is to introduce with the asphalt any of these which aid spreading, lower or control the melting point and are averse to mixing with the asphalt element in the sense of coalescing with it, and which therefore remain as such, free to enter or be absorbed into the absorptive portion of the body material as 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000

soon as the filler layer is melted or brought to a highly loosened condition so as to permit the now highly fluidified, greasy element to leave the denser, sticky element and disappear more or less into the absorptive sawdust or the like. The extent of its disappearance depends upon the speed of the operator, the degree to which the piece is melted, and the relative proportions of the various elements.

5 Suitable by-products of a paraffin base as well as by-products of an asphalt base are found in the market in a large variety of gradations as to hardness, and in fact all their various essential filler qualities and 10 densities, so that it becomes possible to make choices of elements with varying degrees of differences in penetration, or in other words, with different capacities or tendencies for being absorbed. The body materials likewise 15 may be selected with a wide variety of degrees of absorptive capacities. Hence it will be readily understood that the filler piece 20 can be balanced according to the preference of the trade.

25 I have thus explained the above at length to make plain the new principle which I have introduced into the manufacture of these filler pieces. To still further enhance the speed and effectiveness of the filling process 30 with the filler pieces now being explained, I introduce into the filler means for promoting a mechanical or chemical loosening or one which is both mechanical and chemical. For example, the simplest means is to fill the 35 absorptive body particles with water before mixing them into the filler, (as claimed in my copending application Ser. No. 211,157, filed Aug. 6, 1927). In such case the water acts as a stop to prevent the entrance of the 40 petrolatum, for example, or the entrance of any other element of the binder, and at the same time the high heat in the laying process which melts the filler layer for spreading suddenly turns the water into expansive and almost explosive steam which mechanically 45 loosens the filler mass as the water expands and the steam seeks to leave its confinement. Preferably the water is charged with gas-producing chemicals such as sulphate of soda, 50 carbonate of ammonia and the like, which under the action of the heat, generate gas or produce expansion in addition to the steam of the water, thereby producing a still more sudden and effective loosening of the filler.

55 The great heat alone however without these chemicals tends to produce gas in the filler layer because of its sudden effect on the binder, which loosens by expanding, and puffs up the layer, so it spreads more easily, and thereafter becomes a better cushion in the finished 60 shoe-bottom. This expansion or loosening causes a separation of the filler particles and elements which greatly facilitates the work of the operator in the moving of the mass in the direction necessary to fill the cavity prop- 65

erly under the spreading movement of his knife or hand tool. A further application of additional loosening media may be in the form of dry powders sprinkled into the filler as it is being sheeted, such as powdered alum, 70 carbonate of ammonia, sulphate of soda, sulphur, anything which has water of crystallization, sodium chloride, etc. or these may be introduced with the water or stored in the absorptive body material in the form of liquids by themselves. In any case they melt 75 and puff up or loosen because of the gas i. e. gaseous or expansive condition or steam produced by the heat so that they become expanding media for loosening purposes under 80 the action of the high heat when the piece is softened and rendered easily flowable or spreadable. The purpose is to bring about the spreading condition as suddenly as possible so as to avoid prolonged heating (it being 85 desirable to avoid as much heating as possible due to the fact that it is very high heat) and at the same time to use loosening methods and materials, which materials will cease to function as soon as the filler is laid, thereby 90 leaving the filler in its intended tough, dense, stiff and tenacious condition. Moreover, the removal of the water-stop or other barrier from the body material, as stated, and the sudden expansion and porous condition opens 95 the way for absorption of the softer portion of the binder, the petrolatum for example, and accordingly promotes the subsequent hardening and stiffening of the laid piece in the shoe bottom. Broadly stated, any ebullient material, by which I mean anything that will cause the layer to bubble or to expand and become more spreadable, is included within the meaning of the word loosening. Any of the materials mentioned may be 100 used wet or dry in the filler and with or without water or liquid in the body material. For example the carbonate of ammonia breaks down under heat to make gas all through the 105 filler. Sulphur combines with the asphalt and liberates gas. I intend to cover broadly the liberation of gas by heat or chemical reaction as one of the ways of "loosening" the 110 filler. As already stated, the binder, although preferably of the very high melting point mentioned, may be of a lower melting point, and preferably the asphalt is always used although preferably wax tailings (paraffin base) is used with it, but any asphalt 115 may be used and may be modified by softer melting gums, the wide range of which will be apparent from my previous patents. Blown asphalt is elastic and when it melts it becomes slowly fluid, or its viscosity 120 changes gradually under heat. This makes it cling better to the knife even though melted, which is an advantage relied upon for certain purposes, as already explained. I have 125 already explained the advantage of having the body material carry absorbed water, 130

which, when converted into steam, leaves the filler mass porous. On the other hand, the filler material may be made porous originally and provided with starch or any mucilaginous material so that in the shoe factory the piece 5 may be rendered slippery and spreadable by simply being dipped in hot water (this method being covered in my application Ser. No. 242,085 filed December 23, 1927). The desirable porosity may be secured in many 10 ways, the simplest being by putting very little of the tenacious binder (asphalt) in with the comminuted body material so that, because of its strong tenacity, it will, when 15 distended under the sheeting process, hold onto the body particles and yet become attenuated enough to leave pores or minute cavities all through the piece. The piece may be made as firm or rigid as desired for handling 20 and shipping and its spreadability active or always present, or dormant, inoperative or inchoate to be developed in use at the moment of laying. Moreover, the preferred high-heat piece, as distinguished from the cold- 25 laid piece or the low-heat piece, is brought quickly to readiness for spreading, must be then spread at once, and sets immediately. Asphalt is tough and in connection with the comminuted binder material can be spread 30 or forced to yield under strong pressure but yet will cling to the body particles because of its tenacious grip, tensile strength and fine subdivision.

The sulphur permits the further advancement 35 of toughening by semi-vulcanizing the mass and at the same time aiding the porous feature. The asphalts, hydro-carbons or such suitable mineral substances as have a high melting point are then employed or their 40 melting point may be raised to the proper firmness by adding materials to bring the melting point to the degree necessary for the semi-vulcanizing mentioned. For example, to the fluidly heated asphalt or compound, 45 a proportionate amount of powdered sulphur or other finely powdered mineral substance or substances such as slate, talcum, soapstone, plaster of Paris, Paris white, chalk, or lime are added and the mixture heated to about 320°-350° Fahrenheit, the 50 duration varying for heating and semi-vulcanizing according to the fluidity and the amount and kind of vulcanizing agents, as is well known in connection with vulcanizing. 55 The process with sulphur at 320° Fahrenheit is slow, but as the heating is continued, the liquid becomes pasty or the thickness of paste. When in this condition I add powdered cork, wood, charcoal or other similar vegetable, 60 animal or mineral matter, to saturate or fill the hot partially vulcanized paste to a suitable condition in which it can be sheeted into layers between cooled rolls and formed into the standardized filler pieces mentioned. 65 For lightness and cheapness, ground, coarser

grains of all kinds of vegetable matter such as brans from cereals may be added or used as body material, ground bark, in fact anything which gives bulk without undue weight. Ground asbestos may be used. These filler 70 pieces are flexible, stable, or rubber-like, uninfluenced by ordinary conditions of heat, and are light in weight, waterproof, unchangeably flexible, cohesive, non-bunching, porous 75 in the sense of leather, non-heating or non-sweating to the foot in use, and durable without becoming unduly dense and hard. Asphalts and hydrocarbons are non-oxidizing and permanent as binding agents and remain 80 so even when modified by resins, waxes, oils, and gums (of the kinds in my patents). The degree of permanent stickiness of the basic material is varied according to the preference of the trade, but preferably is deadened to a consistency so that when cold the mass resembles more or less a well compounded rubber mass, but not as tenacious although firm, 85 pliable, plastic, bendable, and yet porous as stated and otherwise suitable for footwear in the respects noted, as well as for the purpose of cutting, packaging, shipping, storing and the various processes of handling in shoe factories. In the process of sheeting, the surface is preferably provided with indentations, small corrugations, or depressions to 90 constitute gripping surface and to hold or aid in holding cement or the like for uniting the parts in the shoe-bottom in case such a filler material is used as is not sufficiently adhesive 95 in and of itself. Whenever a more resilient 100 or elastic body is required, I add cottonseed oil, rapeseed, linseed or other vegetable oils whether of a drying or a non-drying nature, their combination and subsequent quasi-vulcanization being accomplished in the vulcanizing treatment of the asphalt materials as 105 already described. The presence of the oils renders the filler mass more resilient, and the amount of the powdered woody, or other body ingredients cooperates to increase or retard the resiliency of the sheeted filler mass. By adding bituminous ingredients which flux with and within the vulcanizable base-forming portion of the binder mass, the rubber 110 qualities and consistency of the filler are controlled so as to effect a so-called semi-vulcanized condition or partially vulcanized condition. This partial vulcanization may also be accomplished by a milder treatment as to 115 heat and the lesser addition of sulphur or other vulcanizing agents. I am distinguishing from real or full vulcanization; the effect is rather a transformation of the heated mass to a more efficacious, pasty nature and condition, resulting in a superior, highly flexible, 120 insulating, water-repellent, light mass at a low cost. The presence of the gas fumes of the sulphur during the prolonged process of heating is the cause of the heated paste becoming porous and sluggishly fluid. 125 130

Although becoming more paste-like and a more efficient binding agent, the binder, because of the sulphur, becomes sufficiently fluid at the stated heat to admit the dry, woody, 5 filler body in a most complete manner, but, because of its partially vulcanized condition, without penetrating into or being absorbed by the body forming powders. When cooled the mass is therefore uniformly compact, tenacious and light, even though no longer fibres have been added. Whenever longer fibres or coarser comminuted body material is added, the sheeted filler is of course correspondingly stronger and tougher. My invention in general which is being set forth in this part of this application is new in employing high heat. This high heat feature of the process is two-fold. First, in conditioning the filler at the start it calls 10 for materials which would not condition in the present filler machines in use today, but require higher heat than the boiling point of water. Second, the high heat is required again for final service to expand and loosen 15 the elements of the filler piece for easy spreading and to release moisture or gas to bubble and raise or loosen the components of the piece momentarily. The high heat at the start makes the material rubbery or tougher 20 and more heat resisting, and the final conditioning it gives speed, simplicity and cleanliness. The speed is not merely in connection with the laying or the work of the operator but is in connection with the further 25 progress of the shoe. The piece being of a nature requiring to receive its heat quickly and strongly, parts with it almost as suddenly. The high heat also by my method is so concentrated, being confined to the small 30 piece, as distinguished from a large bulk or mass of filler in a large machine as heretofore, that the operator is not annoyed with the heat, as he is not obliged to endure a large area of heat radiation, and, because of the 35 high heat arrangement as already explained, it will be evident that no waste occurs as there is no plastic mass left at the end of the day to dry out and be spoiled, and all the necessity for tempering the filler and other 40 present day skilled requirements are eliminated. The high heat involves temperatures and material-conditioning that range beyond the boiling point of water, as distinguished from the temperatures in the moderate heat 45 treatment heretofore common in shoe filler practice, which range below the boiling point of water. The viscosity of the high heat materials mentioned, especially the blown asphalt, makes it practically to concentrate a 50 film of this material on the outer surfaces of the filler layer when it is being sheeted between the wet sheets which act to condense it into a hardened, durable skin or film on the surface as it cools and contracts. Likewise 55 this kind of binder, and again I mention particularly the blown asphalt, develops a fluidity under the high heat treatment which produces a superior stickiness or quick, powerful adherence to the innersole, as well as to the filler piece elements which is of great 60 advantage in the application of the filler piece. The strong tenacity of this high melting binder, also as already explained, makes it possible to have an excess of body material, as compared with previous hot fillers, and thereby produces a mealy or porous layer between the concentrated or condensed outer skins of the binder just explained. The mechanical advantages of this have already been 65 explained. In the eyes of the trade the great 70 advantage of this is in the production of a much lighter weight filler. This total construction provides for great ease in application and a final compacting together of both body and binder materials into a filler layer 75 in a shoe which is non-shiftable, non-bunching, permanently flexible, tough and water-resistant. Another object and advantage of the asphalt type of filler is that it can be used in connection with the German Ago 80 process of making shoes as used in the Michalk apparatus, and it can be used in the Bresnahan compo system, which have recently gone into use in the manufacture of shoes in this 85 country. Both these systems depend largely upon cementing the portions of the innersole, upper and outer sole which come at the bottom of the shoe, and use an acetone cement. My asphalt type of filler, as herein 90 set forth, is not soluble in acetone, whereas 95 the ordinary commercial shoe fillers of the present day cannot be used with these recent systems because their binder dissolves under the influence of the acetone and therefore they run, smear and stain. The variations 100 as to workable quality and consistency previously mentioned tend to render the filler pieces softer, more pliable, and to some extent conformable, when subjected to a downward pressure during the levelling process subsequent to the laying and setting of the filler 105 in the shoe-bottom. 110

The scope of my filler material and standardized units or pieces will thus be seen to be very large in its selection and use of ingredients so that the filler pieces may, if desired, possess qualities which render them self-adhesive by spreading or self-adhesive when subjected to a hot searing contact just before they are laid and set against the shoe-bottom. Even though made extremely stable, the pieces have the advantage of conforming to the varying depths always found in shoe-bottom cavities so as to conform to the downward pressure mentioned in connection with 115 the shoe-bottoming process. The filler piece of any of the kinds thus far mentioned or in fact of any other kind, may have throughout or on one side, or both sides, asphalt or other active or dormant, cementitious matter of 120 125 130

any of the kinds mentioned which are capable of being quickened into active stickiness at the time of application to the shoe-bottom, and then, by being subjected to a sudden heat or to whatever refreshing or quickening influence their particular nature calls for, caused to stick to the shoe-bottom and if spreadable they may be caused thereby to spread under the levelling pressure. A shoe-bottom filler piece made as above stated throughout or solely of blown asphalt has the advantage of permanent flexibility and pliability or non-brittleness and durability when laid in the shoe-bottom, and as a piece before laying is non-sticky and handleable without external protector. Certain species are in my application Ser. No. 228,236 filed Oct. 24, 1927. As already explained, the filler piece is made so as to be externally non-sticky for handling and transportation. The refreshing influence therefore will act as a part solvent or softener for this surface and preferably is of such a nature, as already mentioned, as will disappear soon by evaporation or otherwise after the shoe has been made. The inert materials hasten the sulphur treatment in the case of free flowing kinds of pitches, for instance, by hastening the paste-like consistency in the vulcanizing. To the hot paste I may include with the powdered cork dust, wood dust or the like, tapioca flour, as set forth for instance in my copending application Ser. No. 295,342, filed July 25, 1928, and when sheeted between rolls as stated, and cooled, will possess, in the piece form, a porous interior. Thus the pieces are self-adhesive and may be immersed in hot water and the porosity will allow the tapioca flour or starch, dextrine etc. to soften the pieces and give a slimy, conformable adhesiveness. The porosity not only aids as stated, but it absorbs some of the water and holds the same more or less during the succeeding construction of the shoe, aiding in the better conformation of the parts on the lasts, under the levelling pressure, hammering, etc. and permitting folding at the edge without needing undue force. The sulphate of soda, alum and mucilaginous elements, when used, unite with the plaster of Paris, hydraulic cements, etc. when used, to improve the firm character of the set mass in the shoe-bottom.

This form of my broad invention is advantageous in that it can be sheeted to any reasonable thinness or thickness without any supporting layers, can be died out into pieces having the compactness of leather, the new binding agent supports the layer in its determined shape so that it can be handled etc. and yet can be applied in a softened condition by the operator without the aid of any machine. The pieces, if necessary, can be skived or molded or otherwise mechanically treated. If skived the edges can be folded like other substances and the pieces can be

knicked or compressed or otherwise shaped. The pieces are readily softened. They contain within their structure means for self-adhesion. Also preferably they contain means of the kind mentioned above such as mucilaginous elements, plaster of Paris or the like, for self-firming or toughening while they set and also they can readily be so made that this continues and improves while in their placed positions after they have set. The sheeted material may readily be made of a predetermined firmness or stiffness which is not changed, except temporarily for laying and manipulation, by any action in the compound under the influence of the heat or hot water treatment at the time of use, but is merely softened to a yielding or formative extent, but almost at once, after having been laid and molded or manipulated under the hand of the operator, returns to said condition of predetermined firmness or stiffness.

The practical embodiments of my invention are almost numberless, but as the pieces as such, in their commercial appearance, look about alike, I show, in the following drawings, simply illustrative representations sufficient to add graphically to the remaining presentation and explanation otherwise contained herein. In said drawings,

Figs. 1-4 are fragmentary vertical sectional views of a typical piece, illustrating different details of construction thereof;

Fig. 5 is an edge view of my filler piece;

Fig. 6 shows in bottom plan a forepart of a McKay shoe-bottom which has been filled by the filler piece and method of filling as herein disclosed, the sole having been cut off from the shoe-bottom to reveal clearly the appearance of the laid filler with relation to the other parts after the levelling operation on the shoe-bottom;

Fig. 7 is a vertical cross sectional view through the bottom of a filled Goodyear welt shoe before the sole is laid;

Fig. 8 is a sectional view similar to Fig. 7 of a filled McKay welt bottom before receiving the sole; and

Fig. 9 is a side view partly broken away of an electric hot plate, spatula and filler piece, to illustrate one method of using the filler piece herein set forth.

Referring to the foregoing drawings, the filler piece 1 shown in Fig. 1 comprises a central plastic intermediate layer 2 of spreadable, plastic, compressible shoe filler material and top and bottom covers or supporting layers or carriers 3, 4 which may be of any kind of fabric previously mentioned, as paper, textile webs or the like, which species is duly claimed in my copending application Ser. No. 133,506, filed September 3, 1926, of which the present application is in part a continuation. Fig. 2 shows the piece made with one supporting layer 4 of the kind just mentioned and a top protecting surface 5 of

powdered soapstone, talc, or like inert powdered material, as mentioned in the aforesaid copending application, or any of the crust forming ingredients mentioned in my application Ser. No. 183,302 filed April 13, 1927. Fig. 3 is a similar view illustrating a piece 1 made without a separate cover piece or layer such as presented in Figs. 1 and 2, but of the kind heretofore explained in which the entire piece is composed of relatively homogeneous filler material having a mere skin or thin, tough external surface 6, 7. This surface may be secured in a variety of ways, and preferably consists of the binder itself concentrated or condensed into a hardened, durable skin or film for protecting the piece as an article of commerce. When this surface or skin is composed of a portion of a binder made wholly or in part of asphalt 10 residue of petroleum, it is brought to the required surfacing condition by contacting with the wet canvas in the process of sheeting the plastic filler mass between rolls and layers or webs of wet canvas. The mixed hot filler is passed as a moldable mass between the wet surfaces of two canvas layers driven by heavy rolls and thereby caused to be spread out thin to the thickness required for making the sheet and the pieces, subsequently dried therefrom. The pressure coupled with the chilling effect of the wet canvas and the further cooling effect of the surrounding atmosphere, result in giving a filler layer the desired protective skin or tough 20 surface which, as soon as cold, becomes non-sticky and readily handleable. This surface may be indented as indicated at 8 Fig. 4 to hold cement when desired, or to give a sure gripping surface against the leather or canvas of the shoe-bottom. Said surface 8 may be made by the canvas itself as the piece takes on the roughened appearance made by the impression of the weave of the canvas, or it may be made more pronounced by being 30 subjected to molding surfaces especially chosen for that purpose. In addition, the surface may be sprinkled externally with crust forming materials as indicated at 9 Fig. 5. These may be of the kinds shown at 40 Fig. 2 or may be finely granulated cork or other fibrous, non-absorbent materials, or both. In order to illustrate the comminuted material I have exaggerated the granules out of their true proportion as indicated at 50 which may be taken to represent granules of cork or wood dust or any of the comminuted body materials already mentioned, preferably chosen so as to have some which are porous or absorbent and others non-absorbent 60 and between these are pores 11. The relatively spongy, porous, mealy interior, already explained, results from the choice of materials and the method of manufacture as pointed out, whereby the piece is light and yet tough. Shoe filler is sold by the pound

and the shoe trade is accustomed to reckon the cost by the dozen pairs of shoes, called a "case", so that the lighter the filler is the cheaper to the shoe manufacturer. Hence this element of light weight is an important 70 advantage and an important factor in the invention.

As already stated, the filler piece may be of any suitable shape. Being spreadable it does not need to conform, as made, to the 75 shoe-bottom cavity. In fact no two cavities are exactly alike in shape, which is one reason that it is unnecessary and in fact not advisable that the filler pieces should have the same shape as the cavity. Another reason is 80 that the full efficiency of the filler piece is only developed through the spreading movement of the particles on each other. In Fig. 6 I have shown a filler piece in fully spread position in a McKay shoe, having chosen for 85 this purpose a piece provided with a cover 3 of the shape in my application Ser. No. 192,076, May 7, 1927. If this figure showed a welt shoe, the filler material would be confined within the welt seam, but in the manufacture of a McKay shoe the spreading of the filler material under the levelling pressure is sufficient to fill all the small open 90 spaces formed by the folds or pleats 12. The pressure of the levelling machine squeezes the 95 plastic filler layer outward, as shown in Fig. 6 until stopped by the row of stitches 13. It will be understood that before the sole was removed from the shoe-bottom shown in Fig. 6 the stitches 13 held the sole (not shown), 100 upper 14, and innersole 15 tightly together so that no filler could escape beyond the stitches 13 notwithstanding the severe pressure of the levelling operation. This spreading of the shoe filler, thus extended, to the 105 boundaries of the stitch line 13 so as to fill all the irregular spaces between the sole and the upper formed by the pleats 12, has to take place, if at all, after the sole has been secured on the bottom of the shoe, or, in other words, 110 through the pressure of the leveller. This is a new McKay structure made possible for the first time by my new filler piece and method. In Fig. 7 I have shown a cross section of the bottom of a usual welt shoe indicating by dotted lines at 16 one of my filler pieces which has just been spread to filling position as shown in section at 17. Fig. 8 shows a McKay welt (which may be preferably summarized as a McKay structure having a false welt 18 fastened flat down upon the flat inturned upper 14) which results in giving a fairly well defined shoe-bottom cavity 19 of approximately the same depth as in a welt shoe, and which, because of its better 125 defined cavity boundaries and absence of the usual pleats 12, and open spaces therebetween (as shown in Fig. 6), is readily filled by hand with one of my filler pieces indicated at 20 and spread as indicated at 21. 130

In Fig. 9 I have illustrated the hot method of using my piece which I have explained at length herein, in which illustration a hot plate 22 is represented as provided with electric heating wires 23. The operator places a usual filler knife or spatula 24 flat down on the top 25 of the plate 22 with a filler piece 1 thereon, said knife being halted in proper position by stop 26 and having its handle 27 conveniently resting on a support 28. It will be understood that the plate 22 is preferably rectangular and of a size capable of accommodating the number of knives required for keeping the operator busy but without de-laying appreciably the filler piece thereon after it is heated and ready for use. Let it be supposed that the piece 1 is of the high-heat blown asphalt type. The operator places it on the knife and then places the 20 knife as shown in Fig. 9 with its supported piece down on the hot plate. In a moment the previously dense and more or less rigid, hard filler is loosened by the sudden high heat. As it begins to bubble or expand and 25 rise because of the hot air, gas, steam or other elements causing the ebullition, the operator quickly lifts the knife from its position Fig. 9 and flops it over onto the shoe-bottom as indicated at 16 Fig. 7 or at 20 Fig. 8. The 30 sudden heat has developed the strong stickiness of the asphalt binder so as to cause the piece to cling to the knife sufficiently not to fall off or be thrown askew or otherwise escape from the substantial control of the operator 35 as he flops it over into the shoe-bottom. It will be understood that at this instant the knife blade is at a high heat and the filler piece is also very hot and very sticky so that the operator cannot touch either knife blade 40 or filler piece. Hence it becomes very advantageous that the filler piece shall not readily slide on the knife. The tackiness or sticky tenacity therefore of the particular binder mentioned constitutes an important 45 element in rendering this type of filler piece practical and speedy. The moment the piece touches the bottom of the shoe cavity, the operator instantly brings thereupon the required lateral spreading movement which 50 spreads the highly plastic filler piece from the dotted shape and position Figs. 7 and 8 to the laid position there shown, properly filling the cavity and with its top surface levelled as required. Almost immediately 55 the filler sets, and the operator repeats the process with the next knife, filler piece and shoe.

This method and apparatus have been divided out and filed August 26, 1929, as separate applications Serial Nos. 388,320 and 388,321.

In case the shoe manufacturer wishes to have his McKay shoes filled to the extent shown in Fig. 6, a filler piece of the lower melting variety, as claimed in my applica-

tion Ser. No. 133,506, is selected and placed as indicated at 3 Fig. 6, whereupon the sole is secured in place by the stitches 13 or otherwise. Having applied the sole as stated, usual levelling pressure is brought to bear 70 upon said sole and shoe-bottom, and because of the yielding, compressible nature of my pad-like filler piece, the desired even bottom is secured. The filler piece compresses and yields in whatever direction the cavity 75 and its overlying edge of crimped upper leather and shoe lining require, the semi-plastic or moldable layer 2 between the enclosing, protecting webs or sheets 3, 4 spreading or squeezing out, up, down, or in, 80 as required, and thereby conforming accurately to the differing peculiarities of each shoe-bottom automatically under the severe pressure of the levelling machine. In other words my invention results in producing, in 85 an inexpensive and simple manner, the same proper shape and evenness in a McKay shoe that has heretofore characterized the welt shoe. The pad-like piece allows itself to be compressed and aligned to its surroundings, 90 without requiring any skill or attention from the operator, as this automatic compressing and aligning is accomplished by the regular levelling step in the shoe manufacture, which 95 is always required for molding the sole and bottom.

I wish it understood that I do not undertake herein to set forth any particular preferences as to the shape in which the filler pieces are to be cut as it is merely necessary 100 that they contain enough of the plastic filler material to fill the shoe-bottom according to the requirements of modern shoe manufacture. This leaves an infinite variety of choice as to the particular shape of the piece, from that indicated at 3 Fig. 6 to the shape shown in my copending application Ser. No. 232,279 filed November 10, 1927.

Each piece whether inchoate in the large sheet or piece, or cut or otherwise made, as 110 a small piece or individual leaf, has a self-sustaining sheet-like form and self-maintaining coherency characteristic as an article of manufacture, and with a capacity of expansion in area. This description and definition 115 is intended to be generic to the spreadable leaf, or layer embodiment on the one hand, as more fully set forth and specifically claimed herein, and the non-spreadable but yet extensible leaf, or layer embodiment on 120 the other hand, as herein generically claimed, but claimed as a species in the application of A. H. Avery Ser. No. 212,747 filed August 13, 1927.

As herein shown and described, the piece 125 expands, and preferably spreads or extrudes, laterally outward, i. e. from the center toward and against the periphery of the cavity, although not necessarily, the claim herein being intended to be generic to a structure 130

or piece shiftable in any direction, as for instance inwardly from said periphery toward the center as described and claimed in my copending application Ser. No. 212,018 filed August 10, 1927. The filler piece has a predetermined shape as an article of manufacture, and yet is self-shaping in use and capable of being spread or changed to a different contour or shape and variable thinness under the hands of the operator, or in other words, it is variable in area as well as contour because of its responsiveness to vertical pressure. The wide range or varieties of structural embodiments of my invention is already apparent from the foregoing description. I have already mentioned that the piece is spreadable, and in the laminated embodiment at least one of the layers is preferably spreadable and another preferably fixed or unalterable in shape, and that other layers may be adhesive, active or latent, but as to these various species I refer to the applications where they are claimed as already mentioned. I use the word sheet to mean a broad expanse of material rolled or made thin, but irrespective of whether large or small, and whether parallel sided or not and without preference to whether it is formed into single sizes or pieces for individual shoes, whereas I use the term piece in a broad and different sense to mean simply a single article adapted in size and quantity to the exact requirements of the shoe in the position for which it is intended.

My invention is particularly advantageous in the manufacture of McKay shoes for the reasons already mentioned and also because thereby any of my patented types of plastic filler may be made, as an article of manufacture capable of shipping, handling and storage, into as thin sheets as required for McKay shoes, (not heretofore possible), while at the same time introducing to the McKay shoe all the well recognized advantages of a plastic, moldable, self-shaping shoe filler.

I have already emphasized the factor of having standardized pieces. Each piece has a protective and supporting surface. This surface may be a separate layer, as of paper or other sheet-like fabricated material, with a hard or soft filler interior as desired. On the other hand, instead of having a separate sheet-like surface, said surface may be in the form of a condensed, compressed, plastic skin, made by rolling or pressure or otherwise, and the interior left soft or hard according to composition. This skin may be a hardened layer of the filler material itself, and this may be rendered dense by dusting, impregnating, or coating. This latter treatment may be with inert powder or with flour or dry absorptives or with a combination of any of these materials. The piece may have two protective surfaces, one on each side, and these may be both of the separate, paper-

like or layer type, or both of the condensed, plastic variety, or both of the hardened, coated filler type, or one side may be of one of these types and the other may be of another of the aforesaid. For instance, if the interior is fairly soft, it becomes almost necessary to have at least one side of a tough, sheet-like material such as tough paper or other tough fabric, and the opposite protective surface may then be a hardened layer of filler material, although a separate cover piece would even then be preferable as the soft interior of the piece must depend for its integrity upon the protective outside surfaces, not being self-maintaining alone. Or the piece-shaping, self-maintaining and strength-giving element, layer, or carrier may be internal as already pointed out.

This patent is intended to be foundational or basic in character and accordingly it will be understood that a wide range of mechanical and chemical embodiments is embraced within the scope of its claims, and that most of the previously patented plastic fillers come within the range of availability for the plastic portion of my new filler sheet and the pieces cut therefrom. The various species are claimed in detail in the various applications therefor already mentioned, the generic claims being contained herein.

What I claim is:

1. A shoe bottom filler consisting of a piece made at least in part of plastic material capable of being spread by flowing under pressure and being formed in a consolidated, cohesive unit compacted to self-sustaining consistency as a piece, said piece being of standardized shape and volume, as distinct from being hoppazard or fragmentary, having a volume suitable for filling a single shoe-bottom cavity but greater in thickness and less in area than said cavity, and capable of being spread in the shoe-bottom to the shape and to the reduced thickness and the increased area required for substantially filling said cavity.

2. As an article of manufacture a shoe bottom filler piece which has a volume suitable for filling the bottom cavity of a shoe and is greater in thickness and less in area than said cavity and which is spreadable and adhesive in use but in transportation is cohesive and coherent to the extent of being shape-retaining, and is durable, surface intact and non-adhesive to the extent of being freely handleable and capable of maintaining its shape and integrity as a piece during transportation and until the time of use.

3. A shoe-bottom filler in the form of a piece, as an article of manufacture, having a predetermined volume for filling a single shoe-bottom and which is made at least in part of plastic material capable of being spread by flowing under pressure and is adhesive in use, said piece being compressed,

stable, shape-retaining, and externally non-adhesive under commercial conditions.

4. A shoe-bottom filler piece, which forms a predetermined unit, as an article of manufacture, and is compressed, shape-retaining, non-adhesive, tough, non-stretchable, and stable, under commercial conditions, and is made at least in part of plastic material capable of being spread by flowing under pressure and is adhesive in use.

10 5. A shoe-bottom filler piece, as an article of manufacture, having a predetermined volume for filling a single shoe-bottom, said piece being compressed stable and shape-retaining, externally non-adhesive, and provided with external means for stiffening the piece for handling, and which is made at least in part of plastic material capable of being spread by flowing under pressure and is adhesive in use.

15 6. A shoe-bottom filler piece which is made at least in part of plastic material capable of being spread by flowing under pressure and is adhesive in use but in transportation is cohesive and coherent to the extent of being shape-retaining, and is durable, surface intact and non-adhesive to the extent of being freely handleable during transportation and until the time of use, and which piece is provided with means for stiffening it for handling as a piece.

20 7. An article of manufacture consisting of shoe filler embodied as a shape-maintaining piece, coherent and compressed, standardized in quantity of its filler content to the amount required to fill the intended shoe-bottom cavity and likewise standardized to a less size and shape than said cavity, said article being self-sustaining as a piece for transportation and storage purposes by having a durable and handleable, non-sticky exterior, said piece having a spreadable interior held normally dormant during said transportation and storage.

25 8. A shoe-bottom filler piece which is spreadable and adhesive in use but in transportation is cohesive and coherent to the extent of being shape-retaining, and is durable, surface intact and non-adhesive to the extent of being freely handleable during transportation and until the time of use, and which piece is provided with means for stiffening it for handling as a piece, said piece containing means for increasing the stiffness of the laid filler.

30 9. An article of manufacture consisting of shoe filler embodied as a shape-maintaining piece, coherent and compressed, standardized in quantity of its filler content to the amount required to fill the intended shoe-bottom cavity, and likewise standardized to a less size and shape than said cavity, said article being self-sustaining as a piece for transportation and storage purposes by having a durable and handleable, non-sticky exterior, said

piece having a spreadable interior held normally dormant during said transportation and storage, said piece being adapted to be spread in any direction required for filling the shoe-bottom cavity.

70 10. An article of manufacture consisting of shoe filler embodied as a shape-maintaining piece, coherent and compressed, standardized in quantity of its filler content to the amount required to fill the intended shoe-bottom cavity, and likewise standardized to a less size and shape than said cavity, said article being self-sustaining as a piece for transportation and storage purposes by having a durable and handleable, non-sticky exterior, said piece being spreadable in use to fill the shoe-bottom cavity and then having a self-maintaining coherency characteristic.

75 11. A shape-retaining shoe filler piece, having a self-sustaining form and a coherency characteristic as an article of manufacture, comprising a layer of plastic, adhesive filler material capable of being spread by flowing under pressure.

80 12. A shape-retaining shoe filler piece, having a self-sustaining form and a coherency characteristic as an article of manufacture, comprising a layer of plastic, adhesive filler material capable of being spread by flowing under pressure, said piece having an exterior surface which is sufficiently durable, impervious, non-sticky, and handleable to maintain the piece distinct as an individual piece during ordinary commercial transportation.

85 13. The herein described shoe filler, consisting of material which is at least in part spreadable, formed into a molded and compressed, cohesive, disconnected, individual unit blended to self-supporting compactness, of standardized shape and volume, as distinct from being haphazard or fragmentary, the unit having a volume suitable for filling a single shoe-bottom cavity but greater in thickness and less in area than said cavity, and adapted to be spread in the shoe-bottom to the shape and to the reduced thickness and the increased area required for substantially filling said cavity.

90 14. A shoe-filler piece, which is self-sustaining, compact, impervious, and cohesive so as to be handled and placed as an integral piece in a shoe-bottom, said piece being at least in part adhesive and spreadable, and comprising material in volume to fill the shoe-bottom cavity but less in area than the cavity area and greater in thickness than the cavity thickness and constructed and adapted to be spread in place in said integral-piece condition to said cavity thickness and area in the shoe-bottom.

95 15. A shoe-filler piece, which is molded and compressed to a self-sustaining, dense, impervious, and cohesive condition so as to be capable of being individually handled commercially and then later placed as an integral

125

120

115

110

105

100

95

90

85

80

- piece in a shoe-bottom, said piece comprising, at least in part, adhesive, spreadable material, and having a predetermined volume required to fill the shoe-bottom cavity but less in area than the cavity area and greater in thickness than the cavity thickness and constructed and adapted to be spread in place in said integral-piece condition to said cavity thickness and area in the shoe-bottom.
16. A shoe-filler piece, which is molded and compressed to a self-sustaining, impervious, and cohesive condition so as to be handled and placed as an integral piece in a shoe-bottom, said piece comprising, at least in part, adhesive, spreadable material, and having a predetermined volume required to fill the shoe-bottom cavity but less in area than the cavity area and greater in thickness than the cavity thickness and constructed and adapted to be spread in place in said integral-piece condition to said cavity thickness and area in the shoe-bottom and having means on the outside for keeping said outside substantially dry and non-sticky prior to use.
17. As an article of manufacture, a shoe-bottom filler, having a normally self-sustaining, dense, molded, sheet-like form, and containing an expansible portion of plastic material capable of being spread by flowing under pressure, said expansible portion being responsive to vertical pressure when in a shoe-bottom cavity, to spread into position between the cavity rim and the rest of the filling piece.
18. A shoe-filler piece of sheet-like form, having enclosed within it an adhesive substance capable of being spread by flowing under pressure, and spreadable in response to pressure when in a shoe-bottom cavity to laterally extended position and into adherent relation to the adjacent shoe-bottom surfaces for holding the parts together as a unit.
19. A shoe-filler piece, of sheet-like form, comprising a layer of permanently plastic and adherent shoe-filler material capable of being spread by flowing under pressure, and having an outer skin on at least one side which is substantially non-sticky.
20. A shoe-filler piece for filling shoes, in the form of a thin-sheeted, compacted, self-sustaining and coherent leaf adapted to be handled and placed as an integral self-sustaining piece in a shoe-bottom, said piece including filler elements and having at least one surface resurfaced with said filler elements as described.
21. A shoe-filler piece for filling shoes, having a self-sustaining form and predetermined volume adapted to fill an individual shoe-bottom and capable of occupying as an integral piece the cavity between the outer sole and the innersole, and comprising spreadable material suitable to occupy said cavity and provided with a dry surface protecting means consisting at least in part of dulling powders.
22. A shoe-filler piece for filling shoes, having a self-sustaining form and predetermined volume adapted to fill an individual shoe-bottom and capable of occupying as an integral piece the cavity between the outer sole and the innersole, and comprising material suitable to occupy said cavity and having at least one side normally sticky and provided with a temporary protective means maintaining said sticky surface substantially dry for handling before use.
23. A shoe-filler piece for filling shoes, having a self-sustaining form and predetermined volume adapted to fill an individual shoe-bottom and capable of occupying as an integral piece the cavity between the outer sole and the innersole, and comprising material suitable to occupy said cavity and having at least one side normally sticky and provided with a temporary protective means maintaining said sticky surface substantially dry for handling before use, including comminuted fibrous elements.
24. A filler piece of sheet-like form, comprising a layer of filler material which is plastic, spreadable and adherent to leather, and means rendering the outer faces of said layer substantially dry, smooth and non-sticky but adapted to permit the plastic layers to spread and expose its adherent constituent.
25. An article of manufacture, consisting of shoe-filler embodied as a shape-maintaining piece containing the predetermined quantity required for filling a single shoe-bottom cavity, said piece being made at least in part of plastic material capable of being spread by flowing under pressure, and being adhesive in use and provided with an external protective surface which is relatively frail.
26. An article of manufacture, consisting of shoe-filler embodied as a shape-maintaining piece containing the predetermined quantity required for filling a single shoe-bottom cavity, said piece being spreadable and adhesive in use and provided with an external protective coating adapted to break up and become intermingled with and incorporated into the mass of the filler and so disappear as a coating in the laying of the piece.
27. An article of manufacture, consisting of spreadable shoe-filler embodied as a shape-maintaining piece containing the predetermined quantity required for filling a single shoe-bottom cavity, said piece having its exterior concentrated into a condensed, hardened, durable, film-like skin for facilitating handling and transportation, but adapted to break up when the filler is spread.
28. An article of manufacture, consisting of shoe-filler embodied as a shape-maintaining piece containing the predetermined quan-

5 tity required for filling a single shoe-bottom cavity, said piece being entirely composed of filler material which is spreadable in use and having its external surfaces formed of said filler material concentrated into a condensed, hardened, durable, film-like skin for handling and commercial durability, but adapted to break up when the filler is spread.

10 29. A shoe-filler piece which is shape-maintaining and self-supporting under commercial conditions and spreadable in use, said piece containing binder which under the influence of heat becomes porous.

15 30. An article of the kind described, which is shape-maintaining and self-supporting under commercial conditions, and spreadable in use, and which contains a binder which becomes ebullient under such heat as is necessary for rendering it spreadable in the shoe-bottom.

20 31. A shoe-filler piece which is shape-maintaining and self-supporting under commercial conditions, and spreadable in use, said piece comprising binder and body material united to form a mealy, porous interior and condensed, tough outer skins of the binder.

25 32. A shoe-filler piece which is shape-maintaining and self-supporting under commercial conditions, and spreadable in use, and which comprises a binder containing blown asphalt.

30 33. A shoe-filler piece which is shape-maintaining and self-supporting under commercial conditions, and spreadable in use, said piece comprising comminuted body material and having a high melting point (of the order of 180° to 200° Fahr.) binder united in an impervious, compressed, non-sticky and 35 handleable piece having the volume suitable for filling a single shoe-bottom cavity but greater in thickness and less in area than said cavity.

35 34. A shoe-filler piece which is shape-maintaining and self-supporting under commercial conditions, and spreadable in use, said piece comprising comminuted body material and a binder containing high melting point asphalt mixed together and charged 40 with means for producing gas at the temperatures used in spreading the filler, to effect a sudden loosening of the filler for laying purposes.

45 Signed by me at Boston, Mass., this second day of August, 1928.

50 ANDREW THOMA.